

C. S. PALMER.

METHOD OF MAKING SULPHUR FREE WATER GAS.

APPLICATION FILED JUNE 3, 1918.

1,405,863.

Patented Feb. 7, 1922.

Fig. 2



Fig. 1



Inventor:

Charles S. Palmer,

by his attorney, *Memorial Marton*

# UNITED STATES PATENT OFFICE.

CHARLES S. PALMER, OF PITTSBURGH, PENNSYLVANIA.

## METHOD OF MAKING SULPHUR-FREE WATER GAS.

1,405,863.

Specification of Letters Patent. Patented Feb. 7, 1922.

Application filed June 3, 1918. Serial No. 238,020.

To all whom it may concern:

Be it known that I, CHARLES S. PALMER, a citizen of the United States, residing in Pittsburgh, county of Allegheny and State of Pennsylvania, have invented certain new and useful Improvements in Methods of Making Sulphur-Free Water Gas, of which the following is a specification.

My invention relates to improvements in the manufacture of combustible gases from wood or charcoal and has for its objects the economical and convenient production of a substantially sulphur-free water-gas, the manufacture of charcoal and the water-gas therefrom being preferably carried out by successive operations in the same apparatus, although obviously if desired the successive steps of the manufacture may be conducted in different units of the plant.

The present process of manufacturing water-gas as at present commonly practiced is highly wasteful, in fact about 50 to 60% more coal is consumed in the process merely for maintaining the necessary heat for the water-gas reaction than is necessary, i. e., the present practice consumes about 50% of hard coal or coke for maintaining the reaction temperature, whereas, theoretically but about 30% should be required. A similar loss would occur if charcoal were used in lieu of coal or coke as the fuel treated. Primarily this is due to the wasteful employment of an intermittent air blast for periodically restoring the temperature of reaction as well as being due to the great length of time required when employing the modern retorts in order to heat the contents to the reacting temperature and the consequent serious loss of heat throughout said period by radiation and otherwise.

My invention is fully set forth and described in the accompanying drawings and specification forming a part thereof, in which

Figure 1 is a longitudinal vertical section; and

Fig. 2 is a transverse vertical section along the line 2—2 of Fig. 1.

In the drawings the reference numeral 1 designates the fire-brick walls of the heating chamber having the usual heating flues therein and 2 designates a long narrow

chamber or retort, preferably for example of about 20' x 10' and 8" to 10" wide having a V-shaped bottom, the walls being 55 about  $\frac{1}{2}$ " in thickness. The heating chamber communicates with the usual checker-work of regenerator furnaces positioned below the same (not shown). Preferably such retort is constructed in sections and the same are 60 constructed of a highly refractory, non-oxidizable metal such as ni-chrome steel, though nickel steel or nickel may be also employed in lieu thereof. Suitable poke holes *a* and charging holes *b* are provided at the top of 65 the retort as shown. The lower section preferably has cast iron extensions 3, 3', communicating with a suitable discharge reservoir for any residuum at the end 3 and having a suitable cast iron door 4 covering the 70 end or extension 3'. A gas outlet conduit 5 communicates with the interior of said retort through the said end 3. In the apex of the bottom of the lower section is a longitudinal steam line 6 which has perforations *c* 75 at intervals along the top in order to uniformly admit steam into the bottom of the retort.

Referring to the drawings and the construction shown therein, the operation of the 80 process is as follows:

Sufficient hard wood adapted to yield a good grade of sulphur-free charcoal is introduced through the charging holes to substantially fill the entire retort. Such wood 85 is then subjected to destructive distillation to obtain the volatile products, pyroligneous acid, etc., therefrom by means of heat conducted thereto through the highly conductive, thin, metallic walls of the pipe 5, to 90 containers or reservoirs therefor and the charcoal residuum may be removed into another similar retort through the outlet 3, in order to subject the same to the second stage of the process, but preferably said second 95 stage is conducted in the same retort. The volatile products of destructive distillation so obtained may be suitably scrubbed and otherwise treated in the well known manner to obtain the usual by-products therefrom.

Owing to the high conductivity of the thin walls of my retort, which are preferably about  $\frac{1}{2}$ " thick, and should not exceed  $1\frac{1}{2}$ " in thickness in any event, even the first

stage may be accomplished in a shorter space of time than the process commonly employed at present and as consequence there is but a minimum of fuel and time required for this stage of the process.

In order to produce water-gas from the charcoal residuum of the first stage of the process, the retort is first sufficiently heated by the regenerator furnace gases passing through the flues so as to maintain the mass incandescent by indirect heat only, throughout the second stage of the process, preferably at about 1160° C. Steam is then introduced through the steam-line 6 in sufficient quantities to convert the incandescent coke into water-gas according to the formula  $C + H_2O = H_2 + CO$ . Preferably the steam is superheated, superheating being decided more efficient. Owing to the above stated high heat conductivity of the thin metal walls of my retort, this second stage of the process is completed very rapidly as compared with the usual procedure and the periodically injected hot blasts of atmospheric air are not required in order to maintain the requisite temperatures for the production of water-gas.

"Ni-chrome", and other nickelous alloys consisting principally of nickel, and even nickel itself, unlike iron, ordinarily, while difficultly oxidizable at high temperatures, soon becomes superficially loaded with carbon, when subjected to direct contact with very hot reducing gases having a high carbon content, particularly at temperatures between 1000° and 1100° C. Not only is such carbon physically deposited upon and throughout the exposed surface layer of the metal as graphitic carbon, but also it will be found to be in chemical combination therewith in the form of carbides. The consequence of such loading of nickelous metal with carbon is that it rapidly deteriorates structurally, often becomes weakened to such an extent as to in many cases even crumble to pieces while being subjected to temperatures up to 1100° C., and furthermore its specific heat conductivity becomes very greatly reduced. Under the conditions however to which the nickelous envelope is subjected during the operation of my process, the inner portion thereof is protected from the carbonizing or carbide-forming action of the reducing gases in the retort, because of the fact, as my investigations have shown, that the nickelous portion of the envelope is extremely thin and at the high temperature to which it is subjected, is at least partially pervious to the passage thereof into of the strongly oxidizing external gaseous heating medium, such as the producer-gas and hot air mixture which is preferably employed by me. The result is that the deleterious action of the carbonizing and carbide-forming gas within the retort upon

the inner exposed layer of the envelope is substantially if not entirely, prevented, and instead of the structure of the envelope being seriously weakened and the specific heat conductivity of the envelope being greatly diminished, as would ordinarily be expected by those familiar with the behavior of nickel and its alloys consisting essentially of nickel, the envelope is found to be extraordinarily durable and even after repeated operations of my process herein to retain to a remarkable degree its specific conductivity.

In view of the high conductivity of the walls of the retort and the elimination of the necessity of injecting a blast of heated air thereinto as aforesaid, I am able to obtain from the charcoal a maximum yield of substantially sulphur-free water-gas mixture having a minimum amount of  $CO_2$  and substantially free from nitrogen, i. e., about 5.5% and less than 1% in all cases where the process is properly carried out.

The aforesaid "ni-chrome" alloy approximates in capacity

|         |           |    |
|---------|-----------|----|
| Ni----- | 50 to 60% | 90 |
| Cr----- | 10 to 20% |    |
| Fe----- | 15 to 25% |    |

#### Balance scattering.

Ni-chrome alloy approximates 1200° C., 95 melting point and is relatively non-oxidizable. Moreover, it corresponds substantially to cast iron in tensile strength, heat conductivity and coefficient of expansion.

As above stated, the crux of the invention 100 resides in the indirect heating of the reacting mass by conduction through the non-oxidizable, highly-resistant, thin, metal wall whereby a quick and ready transfer of the large amount of heat required from the outside to the inside of the retort is accomplished, whereas, were the walls constructed relatively thick, say in excess of 1½", even though they were of metal, such transfer of the necessary heat to accomplish the quick 110 conversion of the charcoal into water-gas could not be accomplished, and prolonged heating of the coke by the periodic injection thereinto of hot blasts of air would be necessary in order to prevent the temperature falling below the point at which the water-gas reaction proceeds efficiently, because the reaction  $C + 2H_2O = CO_2 + 2H_2$ , which occurs at lower temperatures, must be avoided in order to obtain an efficient and 120 satisfactory substitute for natural gas.

In my preferred process I also employ ni-chrome steel or other correspondingly highly resistant non-oxidizable metal in the steam line and the superheater, since not 125 only am I thus able to superheat the steam to the reaction temperature when desired, without the destruction of the superheater, but also I avoid the inevitable reduction in temperature which occurs upon the intro-

duction of ordinary superheated steam, which usually is at a temperature considerably in excess of ordinary superheated steam. For example, a steam temperature 5 of 750° to 1100° C., is believed to materially promote the dissociation of the steam, thereby increasing the chemical activity of its elements with the consequence that the formation of hydrocarbons by the interaction 10 of hydrogen of the steam and the carbon (charcoal) is accordingly facilitated. Such a superheater is illustrated in Fig. 1 in which a coil 7 is positioned in a superheating chamber 8, the said chamber being provided 15 with gas inlet and outlets 9 and 10 respectively. In this construction the coil 7 and the entire steam pipe 6 are formed of ni-chrome steel, nickel-steel, nickel or other suitable highly-refractory, substantially 20 non-oxidizable metal alloy consisting essentially of nickel or cobalt.

While nickel itself, when employed for the retort or the superheater piping, forms a thin superficial coating of nickel oxid, I have 25 found that the formation of this crust does not seriously retard the conduction of heat therethrough and furthermore, that said crust does not increase in thickness and cause the deterioration or destruction of the 30 retorts or superheater piping.

As is apparent from the foregoing description, the employment of a highly resistant, non-oxidizable metal retort, having walls not exceeding 1½ inches in thickness, 35 has the following important advantages over a great many of the present water-gas processes as commercially practiced.

First, it avoids the necessity for quenching the charcoal after the removal of the 40 charcoal from the still and prior to its introduction into the water-gas retort, and thereby substantially all of the heat retained in the charcoal at the end of the first stage is conserved, since in my process, as above 45 stated, the water-gas process is preferably conducted in the same retort as the distillation process and immediately following the completion of the latter.

Second, it avoids the necessity for the use 50 of an intermittent air blast to maintain the reacting temperature and thereby prevents the dilution of the gas with large amounts of nitrogen from the heated air blast, and also the maintenance of the uniform temperature 55 enables me to obtain a much more economical and increased yield of gas of a more uniform composition.

Third, the employment of non-oxidizable highly-resistant metallic walls, which 60 should not exceed 1½ inches in thickness, and are preferably ½ inch thick, as a substitute for cast iron or other oxidizable metal retorts or clay and silica retorts now used, permits of the reaction being completed in 65 a much shorter period of time because of the

water-gas reaction being continuous in but a fraction of the time required when the present retorts, which heat extremely slowly, are employed.

Fourth, one of the advantages of employing high-pressure superheated steam at a temperature of 750° C., to 1100° C., is believed to be due to the formation of increased amounts of higher hydrocarbon due to the increased dissociation of the steam, 70 since it is well known that the addition of one or more atoms of carbon or hydrocarbon to a hydrocarbon in many cases very substantially increases the thermal value thereof. This is shown by the following table in 75 which are given the relative thermal units 80 per cubic foot of different hydrocarbons:—

|                | Cal. per kg. | B. T. U. per cub. ft. | 35 |
|----------------|--------------|-----------------------|----|
| $C_2H_2$ ..... | 11,917       | 1,554                 |    |
| $C_3H_6$ ..... | 10,102       | 3,954                 |    |
| $CO$ .....     | 2,436        | 342                   |    |
| $C_2H_6$ ..... | 12,420       | 1,870                 |    |
| $C_3H_8$ ..... | 11,931       | 1,677                 |    |
| $H_2$ .....    | 34,180       | 344                   | 90 |
| $CH_4$ .....   | 13,320       | 1,070                 |    |

In some cases, depending upon the character of the wood and the by-products desired, a small amount of superheated steam can be 95 advantageously injected into the charge in the first distillation stage of the process.

By employing my improved process I can continuously as distinguished from intermittently, produce 500 to 1000 cubic feet of 100 water-gas per square foot of heating surface in every 24 hours, the same approximating the following average composition:—

|                                       |              |     |
|---------------------------------------|--------------|-----|
| $CO$ .....                            | 2% to 10%    | 105 |
| " $C_2H_2$ ," heavy hydrocarbons..... | 0.1% to 0.5% |     |
| $H_2$ .....                           | 50% to 60%   |     |
| " $C_2H_2$ ," Paraffines.....         | 1% to 10%    |     |
| $CO$ .....                            | 20% to 30%   |     |
| N.....                                | Less than 1% | 110 |

Obviously in those cases where the extension 3 is not in communication with the discharge reservoir for the coke residuum resulting from the second or water-gas stage 115 of the process, said extension or end 3 is closed in the same manner as extension 3' by a cast iron door (not shown.)

The employment of platinum, gold, iron (and by iron I include the iron having such 120 carbon content as to come within the range commonly termed steel), as the material of the envelope referred to in the process claimed herein, or, as the material of the retort referred to in the apparatus claimed 125 herein, is specifically disclaimed.

The expression "a metal associated with iron in the 'iron group' in Mendeleef's table and of greater atomic weight than iron," referred to metals which are associated with 130

iron in the group commonly known as the "iron group" consisting of iron, atomic weight 55.84, nickel, atomic weight 58.65 and cobalt, atomic weight 58.97.

5 Having thus described my invention, what I claim and desire to secure by Letters Patent is:—

1. In the manufacture of water-gas from charcoal the process which consists in confining a charge of charcoal substantially free from sulphur and its compounds, in a space having an envelope which consists principally of a metal associated with iron in the "iron group" of Mendeleef's table and 10 of greater atomic weight than iron, said envelope not exceeding  $1\frac{1}{2}$  inches in thickness, being of good heat conductivity and not deleteriously affected when subjected to the action of a mixture of producer gas and air 15 heated to a temperature of 1100° C., for prolonged periods of time, supplying sufficient heat to said charge through said conductive envelope from a strongly oxidizing, highly-heated gaseous medium caused to 20 contact with the outer surface of said envelope, to promote the water-gas reaction in said charge, maintaining said temperature by conduction of heat to said charge through said conductive envelope without the direct 25 introduction to said chamber of substantial quantities of an air blast, simultaneously supplying a sufficient quantity of steam to said charge to effect the water-gas reaction so as to produce a strongly, reducing, highly- 30 heated, gaseous medium in contact with a substantial portion of the inner surface of said envelope.

2. In the manufacture of water-gas from charcoal, the process which consists in confining a charge of wood-charcoal in a space 35 having an envelope which consists principally of a metal associated with iron in the "iron group" in Mendeleef's table and of greater atomic weight than iron, said envelope not exceeding  $1\frac{1}{2}$  inches in thickness, being of good heat conductivity and not deleteriously affected when subjected to the 40 action of a mixture of producer gas and air heated to a temperature of 1100° C., for prolonged periods of time, supplying sufficient 45 heat to said charge through said conductive envelope from a strongly, oxidizing, highly-heated gaseous medium caused to contact with the outer surface of said envelope, to 50 promote the water-gas reaction in said charge, maintaining said temperature by conduction of heat to said charge through said conductive envelope without the direct 55 introduction to said chamber of substantial quantities of an air blast, simultaneously supplying a sufficient quantity of highly super- 60 heated steam at a temperature in excess of 750° C. to said charge, to effect the water-gas reaction, so as to produce a strongly, reducing, highly-heated, gaseous medium in con-

tact with a substantial portion of the inner surface of said envelope and recovering the evolved gas.

3. The process of manufacturing water-gas which consists in confining a charge of wood against the ingress of air in a space having an envelope which consists principally of a metal associated with iron in the "iron group" in Mendeleef's table and of greater atomic weight than iron, said envelope not exceeding  $1\frac{1}{2}$  inches in thickness, being of good heat conductivity and not deleteriously affected when subjected to the action of a mixture of producer gas and air heated to a temperature of 1100° C., heating 70 said charge by means of heat conductivity through said conductive envelope to a temperature sufficient to distill the volatile products from said charge and maintaining said temperature until substantially all of the volatile matter is expelled, withdrawing the liberated volatile substances from said chamber, then conducting sufficient heat through the envelope of said space from a strongly oxidizing, highly-heated, gaseous 75 medium caused to contact with the outer surface of said envelope to elevate the temperature of the residual charcoal therein so as to promote the water-gas reaction, maintaining the said reacting temperature of 80 said coke, while simultaneously introducing steam, without the substantial introduction of oxygen, for a sufficient time to convert the greater part of said coke into water-gas, and thereby produce a strongly reducing 85 highly-heated gaseous medium in contact with a substantial portion of the inner surface of said envelope and recovering the evolved water-gas.

4. In the manufacture of water-gas from charcoal, the process which consists in confining a charge of wood-charcoal substantially free from sulphur and its compounds in a space having an envelope which includes a medium consisting principally of nickel, said envelope being of good heat conductivity and being sufficiently thin to be substantially penetrated into by an external 110 strongly, oxidizing, highly-heated gaseous medium brought into contact with the outer surface of said envelope and also sufficiently thin to permit of the substantial neutralizing of said oxidizing medium of the graphite and carbide-forming tendency of a strongly reducing, highly-heated gaseous 115 medium simultaneously brought into contact with the inner surface of said envelope, said envelope being substantially non-oxidizable when subjected to the action of a mixture of producer gas and air heated to a temperature of 1100° C., supplying sufficient heat to said charge through said conductive envelope, from a strongly oxidizing 120 highly-heated gaseous medium caused to contact with the outer surface of said envelope 125 and recovering the evolved water-gas.

velope, to promote the water-gas reaction in said charge, maintaining said temperature by continued conduction of heat from said gaseous medium through said conductive envelope to said charge without the direct introduction into said chamber of substantial quantities of air, simultaneously supplying a sufficient quantity of steam to said charge to effect the water-gas reaction, so as to produce a strongly reducing, highly-

heated, gaseous medium in contact with a substantial portion of the inner surface of said envelope and recovering the evolved gas.

In witness whereof, I have hereunto set my hand at the city of Pittsburgh, county of Allegheny and State of Pennsylvania, this 1st day of June, 1918.

CHARLES S. PALMER.